

May 7, 1929.

C. C. HALL

1,711,842

EXPANSION JOINT

Filed Nov. 17, 1923



INVENTOR.  
CHARLES C. HALL.

BY

*John C. Hall*  
ATTORNEYS.

## UNITED STATES PATENT OFFICE.

CHARLES C. HALL, OF ALEXANDRIA, INDIANA, ASSIGNOR TO BANNER ROCK CORPORATION, OF ALEXANDRIA, INDIANA, A CORPORATION OF DELAWARE.

## EXPANSION JOINT.

Application filed November 17, 1923. Serial No. 675,369.

This invention relates to an expansion joint for use between sections of paving or the like, such as concrete, cement or other material subject to expansion and contraction.

Expansion joints of this character are inserted between sections of pavement or other surfaces and it is desirable to make them in strips for convenient shipping and handling. The body of the joint, being formed of an asphalt composition, is comparatively soft and plastic and will not retain its formation and shape without a binding or reinforcement of some character. This has heretofore been accomplished in many ways, some of which consist in inserting a flexible metal wire mesh or the like, or interposing and securing together layers of asphalt, paper or burlap, or a layer of asphalt composition between paper or burlap.

It is the object of this invention to produce an expansion joint of the above character by embedding or enclosing therein a plurality of strips of thin wood extending vertically when the joint is in position so as to reinforce and strengthen the material for shipping and handling purposes and give it a substantial vertical rigidity, but permitting horizontal flexibility. To this end the joint is formed with narrow thin wooden strips embedded or enclosed therein at regular intervals so that when applied, the upper edge will be prevented from rolling over, but at the same time such reinforcement will not interfere with its flexibility longitudinally of the reinforcing strips, thereby permitting it to be placed around curves or in any other curved position desired. In other words, when applied, it will be substantially rigid vertically, but flexible horizontally.

Another feature of the invention resides in the method of producing the above-described product as will be hereinafter more fully and specifically set forth.

The full nature of the invention will be understood from the accompanying drawings and the following description and claims:

In the drawings, Figure 1 is a perspective view of the finished product. Fig. 2 is a section taken on the line 2-2 of Fig. 1. Fig. 3 is a section taken on the line 3-3 of Fig. 1. Fig. 4 is a diagrammatic illustration of

the first step in the production thereof. Fig. 5 is a diagrammatic illustration of the second step in the production thereof.

The invention herein comprises an expansion joint consisting of a slab or strip 10 of asphalt mixture possessing desired characteristics as to melting point, ductility, penetration and freedom from constituents that are insoluble in carbon-bisulphide, the asphaltic body having imbedded or enclosed therein at substantially regular intervals sections of narrow thin wooden strips or splinters 11, said wooden strips or splinters being positioned separate from and parallel to each other, as shown in Figs. 1 and 3. Said strips are covered over with the mixture and are so imbedded or enclosed therein as to adhere thereto and form a reinforcement therefor.

It will be observed from Fig. 1 that the body of the joint will have rigidity longitudinally of the strips or splinters of wood, which will be sufficient to permit it to stand between sections of pavement or similar surfaces to be joined, so that the splinters or strips 11 stand vertically, maintain the joint in vertical position and prevent it from rolling over during the work. It will also be observed that by reason of the narrowness of the strips 11, the material will have an appreciable flexibility laterally of the strips or longitudinally of the joint so as to readily permit it to be inserted in curved or rounded positions. This facilitates the shipping, handling and applying of the joints.

The product is produced by melting such asphalt mixture as above described and pouring it upon a metal table top 12, as shown at 13, in Fig. 4. The mixture is poured to an approximate thickness of one and one-fourth inches and before it is chilled, a sheet of thin wood 14 approximately 28 gauge thickness similar to wood prepared for veneers, butterdishes, baskets, etc., is positioned on the surface thereof and pressed down into the melted asphalt by a suitable tool 15 so that said wood veneer or sheet becomes embedded or enclosed therein. When the asphalt material 13 has sufficiently cooled, it is cut into strips of any width desired, usually from three to twelve inches and possibly more. These strips are then put through the rollers 16 mounted in connection with the table bed 18, and rolled to any desired thick-

ness. The rolling elongates the strips of asphalt 13 with sufficient extension in width to cover the ends of the wooden strips 11. Such rolling process and elongation of the asphalt strips 13 will break up the imbedded or enclosed thin wooden sheet, tearing it apart longitudinally of the grain and producing thereby a plurality of separate strips of wood 11, such strips being distributed 10 practically uniformly throughout the length of the rolled product. This product is thereafter cut into any desired length and crated for shipment and use on the job.

It will be understood that the term "veer" as used herein is considered as any type of thin wooden sheets, and the same may be imbedded in the asphalt by applying it to the sides thereof or enclosing it entirely within the same.

20 The invention claimed is:

1. An expansion joint comprising an asphalt composition or equivalent material provided with a plurality of wooden strips imbedded or enclosed therein.

25 2. An expansion joint comprising an asphalt composition or equivalent material

provided with a reinforcement of individual and separated wooden splinters.

3. An expansion joint comprising a strip of asphalt composition or equivalent material provided with a reinforcement of a plurality of wooden strips imbedded or enclosed therein at substantially regular intervals, said strips extending in the same direction and being substantially parallel to 35 each other.

4. An expansion joint comprising a strip of asphalt or equivalent material provided with a reinforcement formed of a thin layer of wood split and separated with the grain 40 and so as to form in substance a plurality of wooden reinforcing splinters.

5. An expansion joint comprising a strip of asphalt or equivalent material provided with a reinforcement comprising a thin 45 layer of wood so positioned in the joint that the joint is flexible transversely of the grain of the wood so as to form in substance a plurality of wooden reinforcing splinters.

In witness whereof, I have hereunto affixed 50 my signature.

CHARLES C. HALL.